

Nov. 28, 1939.

O. H. BIGGS

2,181,291

REFLECTOR BULB LAMP

Filed Dec. 7, 1936



INVENTOR:

Orrick H. Biggs

## UNITED STATES PATENT OFFICE

2,181,291

## REFLECTOR BULB LAMP

Orrick H. Biggs, Beverly, Mass., assignor to Hy-grade Sylvania Corporation, Salem, Mass., a corporation of Massachusetts

Application December 7, 1936, Serial No. 114,562

3 Claims. (Cl. 176—34)

This invention relates to incandescent lamps and particularly to such lamps utilizing a metallic mirror deposited on the bulb of the lamp.

The object of the invention is to provide such a lamp with an internal metallic mirror of high reflectivity, which retains its brightness throughout the usual lamp manufacturing procedure and throughout the life of the lamp. This object is attained by the use of a vacuum-deposited aluminum mirror, covered by a thin transparent film of aluminum oxide, in the bulb of an incandescent lamp filled with an inert gas. At the same time that it protects the aluminum mirror, the oxide film acts as a "getter" to remove water vapor from the atmosphere of the bulb, thus prolonging the filament life.

Previous attempts to use metal films for such a purpose have failed because they either required the shielded evaporation of a metal after the bulb was sealed, in which case a shield remained within the lamp to absorb light, and in which case also it was impossible to secure a sharp cutoff of the reflector edge; or if they used a mirror deposited in the bulb before the lamp was assembled and sealed, they used metals which tarnished when subjected to the heat of exhausting and sealing operations, and which were not protected by a thin transparent film of oxide. The present invention overcomes such defects.

The figure shows a lamp according to the invention. The lamp comprises any usual form of contact base, such as base 1 in the figure; a glass bulb 2 with a restricted neck 6, and a filament 3. The aluminum mirror 4 may be located in any part of the bulb, but is preferably located on the bowl portion as shown, in order to be effective for indirect lighting. The mirror is protected by the thin transparent film 5 of aluminum oxide which covers the mirror. In order to prevent evaporation of the oxide film, a filling of an inert gas is provided in the bulb, preferably at a pressure above half an atmosphere. The bulb, if desired, may have ripples or ridges on its bowl or reflecting portion, for example, as shown in the drawing, to distribute the reflecting light better and to break up any direct image, or may be of some shape suitable for properly distributing the light.

In making a lamp according to the invention, an opaque film of aluminum is deposited on the desired portion of the inside surface of the lamp bulb while the latter is evacuated, preferably as described in copending application Serial Number 691,322 filed September 28, 1933. The film so deposited will form a metallic mirror surface

uncovered by oxide. Air or oxygen is then admitted to the bulb, causing the formation of a thin transparent film of oxide over the surface of the metal. If desired, a heavier protective film of oxide may be formed by means of the well-known anodic processes. The lamp mount may then be sealed into the bulb in the usual manner, for the sealing flame will not affect the aluminum surface, but will merely enhance the oxide coating on it. The bulb may then be exhausted, heated to drive off occluded gases and filled with an inert gas, for example, argon or nitrogen in a manner usual in the art. The oxide-coated aluminum mirror will preserve its reflectivity throughout this process.

Such a lamp finds many uses where the light from the lamp is desired in certain directions and not desired in others particularly for indirect lighting. In many indirect lighting fixtures, a lamp with a metallic mirror coating deposited on the outside of the bulb is now used. The lamp is often placed so that this metal coating is in contact with a grounded fixture. A current can then flow from the hot filament, through the gas inside the bulb, through the hot glass to the grounded mirror. The consequent electrolysis and decomposition of the glass leads to early failure of the bulb. The present invention provides an effective, long-lived mirror surface inside the bulb, thus both insulating the mirror from the grounded fixture and cooling the glass in the region of the mirror, by reflecting the radiation before it hits the glass.

The reflection in the present invention occurs from the surface of the aluminum metal, and not from the surface of the oxide exposed to the atmosphere inside the bulb; that is, the aluminum metal, and not the oxide, reflects the light. To achieve this result, the oxide must be present in a thin translucent layer; and it is preferably present in a transparent layer.

At the same time that it acts as a protection for the aluminum mirror, the oxide film acts as a "getter" to remove any water vapor which may get into the atmosphere of the interior of the lamp bulb, the oxide apparently combining with the water to form the hydroxide. The latter does not spoil the transparency of the oxide film.

This application is a continuation in part of application, Serial Number 623,504, filed July 20, 1932, and of Serial Number 691,322, filed September 28, 1933.

What I claim is:

1. In an electric incandescent lamp, a sealed glass bulb, an opaque light-reflecting layer con-

5

10

15

20

25

30

35

40

45

55

- sisting of substantially pure aluminum over part of the inside surface of the bulb, a transparent protective artificial coating of aluminum oxide covering the aluminum layer, a wire filament within the aluminum-coated portion of the bulb, and a filling of argon at a pressure above half an atmosphere within the bulb.
2. In an electric incandescent lamp, a sealed bulb with a restricted neck portion and a bowl portion, an opaque light-reflecting layer consisting of substantially pure aluminum over the bowl portion only of the bulb, a transparent protective artificial coating of aluminum oxide over the aluminum layer, a gaseous filling of argon at a pressure above half an atmosphere within the bulb, and a wire filament within the aluminum-coated portion of the bulb.

3. In an electric incandescent lamp, a sealed bulb with a restricted neck portion and an approximately hemispherical bowl portion, an opaque light reflecting coating of substantially pure aluminum extending over the entire hemispherical bowl portion of the bulb and a transparent protective artificial coating of aluminum oxide covering the said aluminum, the line of cut-off between the coated bowl and the uncoated portion of the bulb being at the place of maximum bulb diameter perpendicular to the longitudinal axis of the bulb, and a filament positioned entirely within the metal coated bowl portion and disposed in a plane perpendicular to the longitudinal axis of the bulb in order to direct the reflected light out of the bulb.

ORRICK H. BIGGS.